

## UNITED STATES PATENT OFFICE

1,979,250

SOLUBLE, NONCORROSIVE, CUTTING  
COMPOUND

Emil F. Butts, Tacoma, Wash.

No Drawing. Application July 27, 1931,  
Serial No. 553,479

2 Claims. (Cl. 87—9)

This invention relates to the fluid adapted to be poured on the tool and the steel, or other hard material, being cut in a lathe, or other machine tool, for the purpose of keeping the tool and the material being cut from overheating, and to lubricate it.

The objects of my invention are:—To provide a compound which may be shipped and sold in concentrated form, of about the consistency of 10 thick cream, and which may be diluted with water to any desired degree, depending on the speed of cutting and the nature of the materials being used; which will effectively cool and lubricate the tool and the material being cut, thereby 15 preventing damage to the temper of the tool and preventing its too rapid wear; which is noncorrosive; which does not cling excessively to the material and, therefore, is not wasted but which leaves a protective film on the finished material 20 which effectively resists rust from forming on the exposed surfaces; which results in a noticeably cleaner, more highly polished, work than the usual oils used for similar purposes; which very readily mixes with the diluting water; which is 25 free from lumps both in its concentrated and diluted forms and, therefore, does not clog the pipes and passages of the supply system; which does not gum or cake on the tool or metal; and which is cheap and highly efficient.

30 Water is the most effective cooling agent for cooling the tool and the material worked, but it is a poor lubricant and also rusts the surface quickly. Mineral, animal and vegetable oils have a greater lubricating effect on the sliding of the 35 chip or shaving over the lip and face of the cutting tool and will prevent rust, but they have a very poor cooling effect thereon.

I have found that by blending and emulsifying a mineral oil with vegetable oils, in a certain definite proportion, together with a percentage of 40 water, I am able to produce a soluble compound which is a highly efficient cooling agent and lubricant, and which, on drying on the metal, leaves an oily film thereon which greatly resists the 45 formation of rust on the finished surface.

My improved soluble, noncorrosive, cutting compound is formed of the following constituents in substantially the proportions indicated:—

|                            |                |
|----------------------------|----------------|
| Mineral oil                | 71% to 74%     |
| Castor oil                 | 8.25% to 9.5%  |
| Rapeseed oil               | 8.25% to 9.5%  |
| Liquid potassium hydroxide | 8.25% to 9.5%  |
| Sodium carbonate           | 0.60% to 1.25% |

55 The base of the compound is formed of the

mineral oil, which may be of a paraffine base with a gravity of 21 to 26 Baumé; the castor oil ingredient is primarily for the purpose of providing an efficient cooling and lubricating agent; the rapeseed oil is used as a diluent as well as a 60 saponifier; the potassium hydroxide (1370° hydrometer test) is used as an emulsifier; and the sodium carbonate is used to deter or prevent the separation of the ingredients when the compound is diluted with water.

65 My improved compound is prepared in the following manner:—The mineral oil is gradually brought to a temperature of 230° Fahr., and then, while heat is still being added to it, the several ingredients are added in the order given in the 70 above formula, while being slowly stirred until the mass attains a temperature of not over 360° Fahr. The mass is then permitted to cool off to about 240° Fahr., when water is permitted to flow into it. The mass must be continuously 75 stirred to break up any small lumps which may be formed by the water. When enough water has been added to bring its weight to about 140% to 150% of the original weight the product should have a consistency, when cool, of thick cream. 80 The compound may then be barrelled, or poured into cans or other containers, and shipped or stored.

85 The compound may be used by dissolving it in cold water in any desired proportions, usually 85 varying from one part of compound to 2 to 60 parts of water.

Having described my invention, what I claim and desire to secure by Letters Patent, is:—

1. A soluble cutting compound consisting of the 90 reaction products of mineral oil, 71 to 74 parts; castor oil, 8 1/4 to 9 1/2 parts; rapeseed oil, 8 1/4 to 9 1/2 parts; potassium hydroxide, 8 1/4 to 9 1/2 parts; and sodium carbonate 0.6 to 1 1/4 parts; mixed and diluted with water.

95 2. The art of making a soluble cutting compound consisting of heating 71 to 74 parts of mineral oil to a temperature of about 230°; continuing the heating and stirring thereinto 8 1/4 to 9 1/2 parts of castor oil; continuing the heating and stirring thereinto 8 1/4 to 9 1/2 parts of rapeseed oil; continuing the heating and stirring thereinto 8 1/4 to 9 1/2 parts of liquid potassium hydroxide; stirring thereinto 0.6 to 1 1/4 parts of sodium carbonate; heating the mass to about 105 360°; cooling the mass to about 240°; and stirring thereinto about 40 to 50 parts of water.

EMIL F. BUTTS.